

## 1

3,134,669

## COPPER BASE ALLOYS CONTAINING MANGANESE AND ALUMINIUM

Warner Jan de Putter and Gerardus Petrus Knuvers, both of Drunen, Netherlands, assignors to Lips N. V., Drunen, Netherlands, a Dutch corporation

No Drawing. Filed June 11, 1962, Ser. No. 201,292

Claims priority, application Netherlands June 13, 1961  
5 Claims. (Cl. 75—161)

This invention relates to copper base alloys containing manganese and aluminium, and shaped articles, particularly ship's propellers, manufactured from such alloys.

Alloys are known which contain from 2 to 4% iron, 1 to 6% nickel, 3.5 to 9.5% aluminium, 15 to 35% manganese, with the balance being copper and incidental impurities.

Because such alloys have good mechanical characteristics and a good corrosion resistance, they have been proposed as a material for the manufacture of ship's propellers. However, they are relatively expensive and the need is felt for cheaper alloys having at least the same or better characteristics.

With this object in mind, it is now proposed, according to the present invention, to prepare an alloy of this kind having the following composition: 1 to 9% iron, up to 7% nickel and up to 7% cobalt, wherein the total amount of nickel and cobalt taken together is not more than 7%, the three preceding elements when added together amounting to from 3 to 14% of the total weight, 3 to 9% aluminium, 17 to 21% manganese, 1 to 7% zinc, with the balance being copper and the usual impurities.

The alloy prepared according to the present invention has a low melting point, a high impact strength and a very good corrosion resistance, particularly in turbulent sea water.

In the copper alloys of the prior art which contained manganese at a level of between 17 and 21% and which also contained aluminium, which alloys have to satisfy high requirements of mechanical strength, zinc has never been added. It has been the opinion of the experts that the addition of zinc in a higher quantity than that normally encountered as an impurity was unallowable. It has surprisingly been found that zinc, when added to such alloys, has a good effect on several of the above-mentioned characteristics. Moreover, zinc decreases the melting point of the alloy, which decrease is of importance in view of the resulting heat economy.

Additionally, copper-zinc alloys have become known in the art which contains 6 to 20% manganese, 0.1 to 5% iron, 0.1 to 8% nickel and at the most 1.5% aluminium. They are such for bearing sleeves or bushings and similar shaped articles which are subject to sliding friction. The prevailing opinion has been that a higher aluminium content for such alloys would cause the alloys to be much less workable, particularly when cold.

It has been surprisingly discovered that the workability of alloys prepared according to the present invention is quite sufficient for most applications.

The requirement that the total amount of nickel and iron (and possibly cobalt) in the alloys prepared according to this invention should be from 3 to 14% of the total weight is related to the fact that the corrosion resistance in this range is best.

Preferably, the alloys prepared according to this invention contain a total of less than 0.008% arsenic, antimony and/or phosphorus. However these elements when present in higher quantities as usual impurities, do not have much unfavourable influence on the desired characteristics of the alloys.

## 2

Preferably an alloy prepared according to this invention has the following composition: 1 to 6.5% iron, 1 to 6.5% nickel, the two preceding elements taken together constituting 5 to 9% of the total weight, 3 to 9% aluminium, 17 to 21% manganese, 2 to 5% zinc, with the balance being copper and incidental impurities.

More particularly it is preferred to select the composition as follows: 3 to 5% iron, 1 to 3% nickel, 4.5 to 6% aluminium, 17 to 21% manganese, 3 to 5% zinc, with the balance being copper and the usual impurities. This preferred alloy is relatively soft and ductile and has a high elongation.

If it is desired to manufacture an alloy which is relatively hard, the aluminium content is preferably between 6.5 and 9%.

The invention can be realized by melting the components together in a metallurgical furnace in the conventional manner.

## Example I

20 The following elements were melted together in a suitable furnace: 6.06% iron, 2.00% nickel, 5.40% aluminium, 17.52% manganese, 3.31% zinc with the balance being copper and incidental impurities.

25 The alloy was cast into a bar in a sand mold, which bar was suited as a blank for extruding long profiles therefrom. The bar was allowed to cool slowly. Examination of a sample of this alloy gave the following values.

30 Tensile strength ----- 63.2 kg. per square millimeter.

Elongation at rupture ----- 31.6%.

Impact strength (notched):

35 According to Charpy ... 8.1 kg. meter per square centimeter.

According to Izod ----- 5.6 kg. meter per square centimeter.

The deformability and workability at high and normal 40 temperatures and the weldability were good.

## Example II

Following the same manner used in Example I, an alloy 45 was obtained by melting together: 3.0% iron, 2.13% nickel, 4.97% aluminium, 20.1% manganese, 3.92% zinc, with the balance being copper and incidental impurities. The alloy was cast in a sand-cement-mold to a ship's propeller.

50 Examination of a sample of this alloy gave the following values.

Tensile strength ----- 72.5 kg. per square millimeter.

Elongation at rupture ----- 24%.

Impact strength (notched):

According to Charpy ... 7.6 kg. meter per square centimeter.

According to Izod ----- 5.3 kg. meter per square centimeter.

60 The deformability and workability at high and normal temperatures and the weldability were good.

For both the above examples, the corrosion resistance in turbulent sea water flowing at high speed appeared 65 to be excellent.

The above examples only serve to illustrate the invention and it will be clear that the invention is not restricted thereto and that several other embodiments are possible within the scope of the appendant claims.

70 All percentages given in this specification and in the claims are percentages by weight.

What we claim is:

1. A copper base alloy containing manganese and aluminium, having the following composition: 1 to 9% of iron, up to 7% nickel, up to 7% cobalt, nickel and cobalt together not more than 7%, the preceding elements together 3 to 14% of the total weight, 3 to 9% of aluminium, 17 to 21% manganese, 1 to 7% of zinc, with the balance being copper and incidental impurities.

2. An alloy according to claim 1 characterized in that the total amount of arsenic, antimony and phosphorus is less than 0.008%.

3. A copper base alloy containing manganese and aluminium, having the following composition: 1 to 6.5% of iron, 1 to 6.5% of nickel, the preceding elements to-

5

gether constituting 5 to 9% of the total weight, 3 to 9% of aluminium, 17 to 21% of manganese, 2 to 5% zinc, with the balance being copper and incidental impurities.

4. An alloy according to claim 3, having the following composition: 3 to 5% of iron, 1 to 3% of nickel, 4.5 to 6% of aluminium, 17 to 21% of manganese, 3 to 5% of zinc, with the balance being copper and incidental impurities.

5. An alloy according to claim 3, characterized in that it has an aluminium content of 6.5 to 9%.

**References Cited** in the file of this patent

**UNITED STATES PATENTS**

1,962,606 Masing et al. \_\_\_\_\_ June 12, 1934